

## UNITED STATES PATENT OFFICE.

PAUL KESTNER, OF BOULOGNE-SUR-SEINE, FRANCE.

## METHOD OF TREATING WATER.

(No Drawing.

Application filed April 16, 1921. Serial No. 461,925.

*To all whom it may concern:*

Be it known that I, PAUL KESTNER, engineer, citizen of the French Republic, residing at Boulogne-sur-Seine, Department 5 of the Seine, in France, and having P. O. address 113 Boulevard de Strasbourg, in the said city, have invented certain new and useful Improvements in Methods of Treating Water; and I do hereby declare the following to be a full, clear, and exact description of the invention, such as will enable others skilled in the art to which it appertains to make and use the same.

This invention consists in improved metallic media for the fixation of the oxygen of water in apparatus for abstracting gases from liquids.

The fixation of the oxygen dissolved in water is brought about in apparatus for abstracting gases from liquids by the chemical combination of this oxygen with iron filings and turnings, and is represented by the following chemical reactions:



This oxidation is not immediate but requires a certain time to give a quantitative result: the rate of flow of the water in the gas abstracting apparatus is limited to the rate at which the reaction between the iron and the oxygen proceeds in order to obtain effectively the fixation of the oxygen and its complete elimination from the water treated. Consequently, in order to increase the rate of flow of the water in the apparatus for a given quantity of iron, it is necessary to increase the speed of the reaction, and my invention enables this to be attained.

In accordance with the invention a small

quantity of manganese is added to the iron. The manganese acts as a catalyst in the oxidation and combines instantaneously with the oxygen, yielding oxide of iron and protoxide of manganese,  $\text{MnO}$ , capable of oxidizing in turn into dioxide and sesquioxide, which can be reduced again by the iron. The successive reactions which are brought about are as follows:



All these reactions taking place in the water likewise take place between the same oxides in a hydrated state, and constitute a closed cycle, the protoxide of manganese absorbing oxygen continuously and giving it up to the iron until the iron is completely saturated.

The proportion of manganese most favourable for the catalysis is over 5% of the weight of the metal and below 6% of the weight of the iron. The speed of reaction is proportional to the quantity of manganese employed and inversely proportional to the quantity of carbon in the metal.

## Claim:

A method of treating water to de- 75 oxidize it, employing iron or steel filings or turnings containing from 5 to 6 per cent of manganese, the manganese acting as a catalyst in the oxidation of the iron and increasing considerably the speed of the re- 80 action which takes place.

PAUL KESTNER.